

# UNITED STATES PATENT OFFICE.

FRANCIS L. BIRD, OF ELIZABETH, NEW JERSEY.

## COMPOSITION FOR DRY-STAMPING, &c.

SPECIFICATION forming part of Letters Patent No. 288,199, dated November 13, 1883.

Application filed June 9, 1883. (No specimens.)

*To all whom it may concern:*

Be it known that I, FRANCIS LUCAS BIRD, a citizen of the United States, and a resident of the city of Elizabeth, Union county, New Jersey, have invented a new and useful composition of matter to be used for dry-stamping, printing, or picturing, with perforated patterns, stencil-plates, or cut-designs upon woolen, silk, velvet, cotton, and other materials, to of which the following is a specification, viz:

My composition consists of powdered aluminium bronze and powdered white-metal bronze, which latter is known in the trade as silver-composition bronze, mixed with an equal quantity, in weight, of pulverized gum, such as gum-dammar, rosin, or a similar gum. These ingredients are to be thoroughly mixed together. The specimen contains the following proportions, viz: twenty-five per cent., in weight, of gum-dammar; twenty-five per cent., in weight, of rosin; twenty-five per cent., in weight, of aluminium bronze; and twenty-five per cent., in weight, of white-metal bronze.

In using the above-named composition the process is known as "pouncing," and is done by placing the pattern (rough side up, if parchment or paper patterns are used,) stencil-plate, or cut design on the material to be stamped, printed, or pictured, as the case may be, with weights placed at the corners to keep from slipping. Make a distributor by covering a small block of wood with a piece of fine felt. Place a small portion of the composition upon some hard smooth surface, and rub the distributor well into the composition, and shake off the loose powder from the distributor. Then rub the distributor over the perforations in the plates or designs until the pattern is clearly marked on the material. Then carefully remove the pattern, lay a piece of thin paper over the pictured design, and pass a hot iron over it. (For stamping on velvet hold the back of the stamped velvet against the face of the iron until the gum in the composition is melted.) The iron should be as hot as possible without scorching the material. (Thin material may be ironed on the back.) This will melt the gum in the composition and fasten the design to the material. The material then, as stamped, printed, or pictured, is immediately ready for use.

This composition is applicable for goods of all colors; is very durable, and maintains its

bright and shining color. It is not affected by the heat or dampness of the weather. 5

A great want has long been and is now felt for some powder that will stamp dark-colored dry-goods and hold the design upon the material until embroidered. A preparation called "French oil" is now generally used for this purpose. This preparation is made from white zinc and boiled linseed-oil, with a drier added; but it is troublesome to make and is dangerous to use on account of its indelible nature. The parchment pattern that has been used with it must have one or more washings in benzine or naphtha after using, in order to free the holes from the oil, and if any of the oil is spilled, or a mistake is made in the stamping, the material may be ruined. Upon 7 goods of a light color the common preparation used is gum and prussian-blue; but this is only applicable to light-colored materials.

Many attempts have been made to use some light-colored substances other than bronze in connection with gum for stamping with the same patterns that have before been used with prussian-blue; but all such attempts fail, (see Ingalls' Manual, page 9, published by J. F. Ingalls, of Lynn, Massachusetts,) because either 8 the prussian-blue remaining upon the pattern contains such strong coloring properties that when the heat is applied it overcomes the white and robs it of its marking power, or because the white material used is destroyed 8 by the coloring matter in the goods. My composition can be used with patterns upon which prussian-blue has been used, or any marking preparation in use, provided the patterns are dry. 9

I am not aware that any composition of powdered aluminium bronze and powdered white-metal bronze have been used with gum for the purpose of stamping, printing, or picturing. 9

What I claim, and desire to secure by Letters Patent of the United States, is—

A composition of gum or gums, including rosin, with powdered aluminium bronze and powdered white-metal bronze combined. 1

In testimony that I claim the foregoing as my invention I have signed my name, in presence of two witnesses, this 8th day of June, 1883.

Witnesses: FRANCIS L. BIRD.

THEODORE F. ENGLISH,  
JOHN J. LOWDEN.